

Dec. 23, 1958

J. J. HEGER ET AL

2,865,740

PRECIPITATION-HARDENING NONMAGNETIC-FERROUS ALLOYS

Filed June 23, 1954

5 Sheets-Sheet 1

FIG. 1.



EFFECT OF VANADIUM IN A 0.40 PERCENT CARBON STEEL

INVENTORS:

JAMES J. HEGER,  
JOHN M. HODGE and  
RAYMOND SMITH,

BY: *Donald G. Dalton*  
their Attorney.

Dec. 23, 1958

J. J. HEGER ET AL

2,865,740

PRECIPITATION-HARDENING NONMAGNETIC-FERROUS ALLOYS

Filed June 23, 1954

5 Sheets-Sheet 2

FIG. 2.



EFFECT OF ALUMINUM IN A 0.34 TO 0.45 PERCENT CARBON  
AND 0.40 TO 0.52 PERCENT VANADIUM STEEL

INVENTORS:

JAMES J. HEGER,  
JOHN M. HODGE and  
RAYMOND SMITH,

BY: *Donald G. Dalton*  
their Attorney.

Dec. 23, 1958

J. J. HEGER ET AL

2,865,740

PRECIPITATION-HARDENING NONMAGNETIC-FERROUS ALLOYS

Filed June 23, 1954

5 Sheets-Sheet 3

FIG. 3.



EFFECT OF CHROMIUM IN A 0.40 PERCENT VANADIUM  
AND IN A 0.75 TO 1.0 PERCENT VANADIUM STEEL

INVENTORS:  
JAMES J. HEGER,  
JOHN M. HODGE and  
RAYMOND SMITH,

BY: Donald G. Dalton  
their Attorney.

Dec. 23, 1958

J. J. HEGER ET AL

2,865,740

PRECIPITATION-HARDENING NONMAGNETIC-FERROUS ALLOYS

Filed June 23, 1954

5 Sheets-Sheet 4

Fig. 4



EFFECT OF VANADIUM IN A 5.0 PERCENT CHROMIUM  
AND 0.40 TO 0.50 PERCENT CARBON STEEL

INVENTORS:

JAMES J. HEGER,  
JOHN M. HODGE and  
RAYMOND SMITH,

BY: *Donald G. Dalton*  
*their Attorney.*

Dec. 23, 1958

J. J. HEGER ET AL

2,865,740

PRECIPITATION-HARDENING NONMAGNETIC-FERROUS ALLOYS

Filed June 23, 1954

5 Sheets-Sheet 5

FIG. 5.



EFFECT OF CARBON IN A 5.0 PERCENT CHROMIUM  
AND 1.0 PERCENT VANADIUM STEEL

INVENTORS:

JAMES J. HEGER,  
JOHN M. HODGE and  
RAYMOND SMITH,

BY: *Donald G. Dalton*  
their Attorney.

1

2,865,740

## PRECIPITATION-HARDENING NONMAGNETIC-FERROUS ALLOYS

James J. Heger, Bridgeville, and John M. Hodge and Raymond Smith, Pittsburgh, Pa., assignors to United States Steel Corporation, a corporation of New Jersey

Application June 23, 1954, Serial No. 438,816

9 Claims. (Cl. 75—123)

This invention relates to austenitic ferrous alloys that can be hardened by precipitation-hardening heat treatments and precipitation-hardened articles formed therefrom.

There are numerous applications for austenitic steels that may be precipitation- or age-hardened whereby the necessity for cold working to achieve hardening may be avoided. While the use of phosphorus, titanium and other elements to achieve age-hardening in austenitic alloys of the high chromium type has been suggested, such ingredients have certain undesirable characteristics which render the alloy either unsuitable for many applications or have an adverse effect on the hot working qualities thereof.

The high chromium "stainless" type austenitic alloys are widely used for high temperature applications due to their oxidation resistance and in many other instances where resistance to corrosion is a factor. There is however also a demand for austenitic, precipitation-hardenable alloys which contain either no chromium or relatively small amounts thereof. One particular use for the latter is retainer rings for large electrical generators. In order that such generators be not too massive, the steels used in their construction must have high strength and also must be nonmagnetic to prevent overheating by eddy currents. Obviously, cold work is unsuitable for hardening such articles.

It is accordingly an object of this invention to provide age-hardenable, austenitic steels which have unimpaired working properties and no harmful inclusions therein.

It is a further object of this invention to provide chromium containing austenitic steels which are age-hardenable.

It is another object of the present invention to provide low-nickel, manganese-nickel austenitic steels which are age-hardenable and also possess good hot and cold working qualities.

The foregoing and further objects will become apparent from the following specification when read in conjunction with the attached drawings wherein Figures 1 through 5 are graphs, the ordinates of which show the (DPH) hardness values of steels containing the varying amounts of alloying elements shown on the abscissas. The broken

2

horizontal line in each figure indicates the nominal annealed hardness of the steel.

We have discovered that the objects of this invention can be achieved by properly adjusting the elements carbon and vanadium in such austenitic steels and, if further age-hardening effects are desired, by the addition of aluminum thereto within certain critical amounts. Provided these elements are added within the ranges herein-after disclosed, the steel can then be age-hardened by first heating it to a temperature high enough to dissolve the vanadium carbides, which form in the steels of our invention, and place such carbides in solution, cooling so as to retain the vanadium and carbon in solution and then reheating to a temperature above room temperature and below the temperature at which the vanadium carbides can be placed in solution. At this intermediate temperature a precipitation occurs and the resulting precipitate markedly increases the strength and hardness of the material.

In our steels the austenitic structure is preferably produced by suitable combinations of the elements manganese and nickel. Manganese may be present in amounts up to 16%; higher amounts could possibly be used so far as this invention is concerned except for steel melting difficulties which are associated with such higher amounts. Nickel may be present in amounts up to about 12%; high amounts are uneconomical. While the austenitic structure may be produced by additions of manganese alone or by additions of nickel alone, we have preferred to use combinations of manganese and nickel in which the nickel content is as low as possible for economical reasons. A small nickel content of the order of 2 to 4% is ordinarily preferred to enhance the hot working qualities.

In preparing our steels, at least .25% carbon is required. Considerably higher amounts of this element may be used, however it should not exceed about 1% as forging difficulties are encountered above this amount. Vanadium should be above about .30%, preferably above .40% and may be present up to about 3%, the upper limit being dictated largely by economic reasons.

We have also discovered that certain additions of the elements chromium and molybdenum may be made to our steels for their normal effect on the corrosion or oxidation resistance of the steel without adversely affecting the precipitation hardening characteristics thereof and within certain limits a beneficial effect can be obtained. Aluminum can be added to further enhance the hardening effects.

Other elements such as phosphorus, silicon and sulphur may be present within ordinary commercial limits, i. e., .04% maximum phosphorus, .035% maximum sulphur and 1.0% maximum silicon. Other elements may be present in residual amounts, the balance of the alloy being iron.

Specific examples of carbon steels that come within the scope of our invention are shown in the following Table I:

Table I  
EFFECT OF CARBON AND VANADIUM

| Steel No. | C   | Mn    | Ni    | Si  | Cr    | Al    | V     | Annealed Hardness (DPH) | Hardness (DPH) After Aging For 64 Hrs. at 1,200° F. |
|-----------|-----|-------|-------|-----|-------|-------|-------|-------------------------|-----------------------------------------------------|
| 1.....    | .40 | 14.00 | 9.57  | .40 | .007  | ..... | ..... | 140                     | 140                                                 |
| 2.....    | .39 | 13.20 | 13.23 | .35 | .07   | ..... | .28   | 140                     | 240                                                 |
| 3.....    | .38 | 14.20 | 9.56  | .47 | .38   | ..... | .26   | 155                     | 256                                                 |
| 4.....    | .55 | 15.00 | 9.45  | .36 | ..... | ..... | .38   | 154                     | 236                                                 |
| 5.....    | .38 | 15.10 | 10.02 | .57 | .19   | .11   | 1.20  | 162                     | 310                                                 |

## 3

In this table, we have listed the hardness after aging of a series of austenitic manganese-nickel steels having various amounts of carbon and vanadium. As will be noted, steel No. 1 which contains carbon but which does not contain vanadium will not age-harden, whereas the 5 steels which contain over .30% vanadium and over .25% carbon undergo a considerable increase in hardness to above 230 DPH upon heating for 64 hours at 1200° F. This increase in hardness that occurs on heating is related to the amount of vanadium and the amount of carbon that are present in the steel, a certain minimum of each being required if a definite degree of hardening is to be obtained. Preferably to make the steel sufficiently age-hardenable and to make the heat treatment economical a minimum of about .30% vanadium and .25% carbon should be present.

In order to be satisfactory as retaining rings in generators, the material must be capable of being hardened to a minimum of DPH hardness of 300. As will be noted from the examples given in Table I, this minimum DPH hardness of 300 DPH can be achieved by having about .40% carbon and 1.00/1.20% vanadium in the steel. However, vanadium is a very expensive element and, accordingly, other methods were sought to make this steel age-hardenable to the prescribed DPH hardness of 300. We have discovered that additions of aluminum to a steel containing nominally about .30% carbon and .40% vanadium will produce steels that are capable of being aged to DPH hardnesses well in excess of 300.

The effects of aluminum on steels containing varying carbon and varying vanadium contents and also chromium and molybdenum are given in Table II and also shown on the graph of Figure 2.

Table II  
EFFECT OF ALUMINUM

| Steel No. | C   | Mn    | Ni    | Cr   | Al   | V   | Mo  | Hardness (DPH) After Aging For 64 Hrs. at 1,200° F.  |
|-----------|-----|-------|-------|------|------|-----|-----|------------------------------------------------------|
| 6         | .34 | 15.00 | 10.02 |      | .62  | .47 |     | 172                                                  |
| 7         | .40 | 15.10 | 10.12 |      | 1.16 | .47 |     | 263                                                  |
| 8         | .36 | 15.00 | 10.00 |      | 2.07 | .50 |     | 292                                                  |
| 9         | .38 | 15.00 | 10.02 |      | 3.48 | .50 |     | 430                                                  |
| 10        | .40 | 15.25 | 9.51  |      | 3.07 | .46 |     | 323                                                  |
| 11        | .41 | 14.80 | 9.52  |      | 3.04 | .41 |     | 355                                                  |
| 12        | .40 | 16.05 | 9.98  |      | 2.90 | .43 |     | 345                                                  |
| 13        | .40 | 16.04 | 9.96  |      | 3.10 | .52 |     | 410                                                  |
| 14        | .34 | 16.47 | 9.99  |      | 2.84 | .53 |     | 392                                                  |
| 15        | .42 | 15.80 | 10.95 |      | 2.94 | .42 |     | 359                                                  |
|           |     |       |       |      |      |     |     | Hardness (DPH) After Aging For 116 Hrs. at 1,200° F. |
| 16        | .33 | 12.90 | 10.07 | 4.58 | 2.97 | .31 |     | 280                                                  |
| 17        | .41 | 13.65 | 10.01 | .079 | 3.39 | .28 | .90 | 435                                                  |
| 18        | .39 | 13.40 | 9.99  | 5.05 | 3.39 | .28 | .89 | 445                                                  |

As will be noted, with an aluminum content above about 3%, .40% minimum carbon content and a .40% minimum vanadium content, the steel will consistently be capable of being age hardened to a DPH hardness of well in excess of 300. However, as shown in Figure 2, aluminum contents between the residual amounts associated with substantial deoxidation and about 1.2% have a harmful effect on age-hardening. Accordingly, if used, this element should be present in amounts over about 1.2%. Increasing amounts thereof are beneficial so far as age-hardening is concerned but other qualities of the steel are seriously and adversely affected if the aluminum exceeds about 4%.

## 4

We have also discovered that additions of about 4-5% chromium to our vanadium-carbon austenitic and thus nonmagnetic steels also will produce a steel that can consistently be age-hardened to a minimum DPH hardness of 230. See for example Table III and Figure 3.

Table III  
10 EFFECT OF CHROMIUM IN A 0.40% C-0.40% V STEEL

| Steel No. | C   | Mn    | Ni | Cr   | V     | Hardness (DPH) After Aging For 64 Hrs. at 1,200° F. |     |
|-----------|-----|-------|----|------|-------|-----------------------------------------------------|-----|
| 19        | .39 | 9.9   |    | 4.04 | 1.98  | .42                                                 | 287 |
| 20        | .38 | 10.50 |    | 4.20 | 4.20  | .41                                                 | 302 |
| 21        | .38 | 8.70  |    | 4.10 | 8.00  | .43                                                 | 260 |
| 22        | .42 | 7.90  |    | 3.80 | 12.01 | .40                                                 | 230 |

20 EFFECT OF CHROMIUM IN A 0.40% C-0.75/1.0% V STEEL

| Steel No. | C   | Mn   | Ni | Cr   | V     | Hardness (DPH) After Aging For 64 Hrs. at 1,200° F. |     |
|-----------|-----|------|----|------|-------|-----------------------------------------------------|-----|
| 23        | .42 | 8.00 |    | 4.08 | 5.05  | .77                                                 | 387 |
| 24        | .45 | 8.30 |    | 3.80 | 10.60 | 1.03                                                | 402 |
| 25        | .46 | 8.50 |    | 3.80 | 12.50 | 1.03                                                | 387 |
| 26        | .43 | 7.60 |    | 4.70 | 14.60 | .99                                                 | 364 |
| 27        | .45 | 8.10 |    | 4.10 | 16.70 | 1.08                                                | 345 |

30 This table further shows that with a .75% to 1.0% vanadium content, high chromium contents can be used without seriously affecting the age-hardening properties.

35 The effect of vanadium and carbon contents with the preferred 4-5% chromium content are shown in Figures 4 and 5 and tabulated in Tables IV and V.

40 Table IV  
EFFECT OF CARBON IN A 5% Cr-1% V STEEL

| Steel No. | C   | Mn   | Ni   | Cr   | V    | Hardness (DPH) After Aging For 64 Hrs. at 1,200° F. |
|-----------|-----|------|------|------|------|-----------------------------------------------------|
| 28        | .15 | 9.0  | 7.0  | 5.00 | 1.00 | 260                                                 |
| 29        | .25 | 9.0  | 7.0  | 5.00 | 1.00 | 350                                                 |
| 30        | .35 | 9.0  | 7.0  | 5.00 | 1.00 | 373                                                 |
| 31        | .43 | 8.20 | 7.70 | 4.33 | .86  | 363                                                 |
| 32        | .53 | 8.40 | 4.80 | 4.56 | 1.07 | 410                                                 |
| 33        | .58 | 8.20 | 4.80 | 4.52 | 1.02 | 406                                                 |
| 34        | .57 | 8.20 | 5.74 | 4.49 | 1.02 | 392                                                 |

55 Table V  
EFFECT OF VANADIUM IN A 4.0/5.0% Cr-4.0% C STEEL

| Steel No. | C   | Mn   | Ni   | Cr   | V    | Hardness (DPH) After Aging For 64 Hrs. at 1,200° F. |
|-----------|-----|------|------|------|------|-----------------------------------------------------|
| 35        | .41 | 9.80 | 4.02 | 3.98 | .53  | 327                                                 |
| 36        | .47 | 9.60 | 4.07 | 4.00 | .25  | 273                                                 |
| 37        | .52 | 5.80 | 5.75 | 4.45 | .80  | 402                                                 |
| 38        | .44 | 7.40 | 3.91 | 4.79 | .75  | 382                                                 |
| 39        | .44 | 8.70 | 6.26 | 4.85 | .75  | 373                                                 |
| 40        | .42 | 8.00 | 4.08 | 5.05 | .77  | 387                                                 |
| 41        | .43 | 8.20 | 7.70 | 4.33 | .86  | 364                                                 |
| 42        | .53 | 8.40 | 4.82 | 4.56 | 1.07 | 410                                                 |
| 43        | .50 | 9.60 | 3.73 | 4.63 | .38  | 318                                                 |

70 75 Table VI shows that with higher vanadium contents, chromium contents up to 20% can be tolerated without seriously affecting the age-hardening.

5  
Table VI

## EXAMPLES OF THE STEELS HAVING HIGH Cr CONTENTS

| Steel No. | C   | Mn   | Ni    | Cr    | V    | N     | Hardness (DPH) After Aging For 64 Hrs. at 1,200° F. |
|-----------|-----|------|-------|-------|------|-------|-----------------------------------------------------|
| 44        | .16 | 9.20 | 11.72 | 19.56 | 2.45 | .12   | 245                                                 |
| 45        | .11 | 8.00 | 4.06  | 15.70 | 2.04 | .12   | 260                                                 |
| 46        | .11 | 7.80 | 3.98  | 15.65 | 2.04 | .13   | 280                                                 |
| 47        | .23 | 7.70 | 4.06  | 16.47 | 1.07 | ----- | 260                                                 |
| 48        | .22 | 8.60 | 7.99  | 16.75 | 2.04 | ----- | 350                                                 |
| 49        | .22 | 7.10 | 4.44  | 15.44 | 1.99 | .11   | 355                                                 |
| 50        | .22 | 1.38 | 11.66 | 17.50 | 2.86 | .12   | 276                                                 |
| 51        | .22 | 9.00 | 11.59 | 19.07 | 2.04 | ----- | 315                                                 |
| 52        | .27 | 8.80 | 11.63 | 19.29 | 2.50 | ----- | 319                                                 |
| 53        | .22 | 4.40 | 11.79 | 19.29 | 2.04 | ----- | 306                                                 |
| 54        | .22 | 4.40 | 11.99 | 18.28 | 2.50 | ----- | 280                                                 |
| 55        | .33 | 7.50 | 4.30  | 16.54 | 1.02 | ----- | 323                                                 |
| 56        | .36 | 8.00 | 3.98  | 16.72 | 2.04 | ----- | 410                                                 |
| 57        | .35 | 4.00 | 12.00 | 18.03 | 1.99 | ----- | 298                                                 |
| 58        | .34 | 1.00 | 12.00 | 18.54 | 2.35 | ----- | 286                                                 |
| 59        | .35 | 1.00 | 12.00 | 18.95 | 2.04 | .11   | 327                                                 |
| 60        | .31 | 8.00 | 4.00  | 12.29 | 1.99 | .11   | 373                                                 |

Additions of up to 4% molybdenum have been made to the steels of our invention, not only without harm to the aging reaction but with apparently a slightly beneficial effect thereon. Amounts over 4% may be used provided the austenite formers are adjusted within the ranges set forth above to offset the ferrite forming tendency of the molybdenum and maintain the steel in an austenitic condition. Under some circumstances, molybdenum may be desired for such purposes as increasing high temperature, strength, etc. The effects of molybdenum are shown in the following Table VII:

Table VII

## EXAMPLES OF STEELS CONTAINING MOLYBDENUM

| Steel No. | C   | Mn    | Ni    | Cr    | V    | Mo   | Hardness (DPH) After Aging For 64 Hrs. at 1,200° F. |
|-----------|-----|-------|-------|-------|------|------|-----------------------------------------------------|
| 61        | .42 | 9.55  | 4.03  | ----- | .35  | .98  | 302                                                 |
| 62        | .41 | 13.56 | ----- | 11.20 | .44  | 1.00 | 276                                                 |
| 63        | .51 | 7.80  | 7.70  | 12.36 | 1.07 | 1.02 | 382                                                 |
| 64        | .50 | 8.30  | 7.71  | 5.43  | 1.02 | 1.02 | 430                                                 |
| 65        | .50 | 7.90  | 7.84  | 5.85  | .92  | 1.95 | 440                                                 |
| 66        | .47 | 9.50  | 8.39  | 5.67  | 1.02 | 3.00 | 411                                                 |
| 67        | .45 | 10.30 | 7.77  | 4.28  | 1.02 | 3.95 | 424                                                 |

In all of the steels listed, it will be noted that the manganese-nickel contents vary over a considerably wide range, thus showing that the amounts of these elements are not critical insofar as age-hardening is concerned, but are present merely to make the structure of the steel austenitic.

As before stated, to age harden the steels of our invention, they are first solution annealed at a temperature sufficiently high to place the vanadium carbides in solution. As shown in the following Table VIII, a temperature at least about 2000° F. should be used. Higher temperatures below the fusing temperature of the steel can be used. However, in view of increased heating costs, scale losses, and other undesirable effects associated with heating to very high temperatures, we prefer to use temperatures below about 2300° F.

Table VIII

## EFFECT OF SOLUTION ANNEALING TEMPERATURE

| Steel No. | C   | Mn   | Ni   | Cr   | V    |
|-----------|-----|------|------|------|------|
| 32        | .53 | 8.40 | 4.80 | 4.56 | 1.07 |

| Solution Annealing Temp. (° F.) | Hardness (DPH) After Aging For 8 Hours at 1,300° F. |
|---------------------------------|-----------------------------------------------------|
| ½ hr. at 2,000                  | 341                                                 |
| ½ hr. at 2,050                  | 368                                                 |
| ½ hr. at 2,100                  | 387                                                 |

10 The effects of aging temperatures following solution annealing at 2170° F. for ½ hour are shown in the following Table IX.

Table IX  
EFFECT OF AGING TEMPERATURE OF MATERIAL SOLUTION ANNEALED AT 2170° F. FOR ½ HR.

| Aging Treatment      | Hardness (DPH) |
|----------------------|----------------|
| 64 Hrs. at 1,200° F. | 392            |
| 8 Hrs. at 1275° F.   | 373            |
| 8 Hrs. at 1300° F.   | 377            |
| 8 Hrs. at 1350° F.   | 364            |
| 8 Hrs. at 1375° F.   | 350            |

25 Good results can be obtained by a long time, 64 hour treatment at 1200° F. However, shorter times at higher temperatures up to about 1350° F. can be used. Other experiments have indicated that temperatures of at least 1100° F. must be used.

30 While we have shown and described a number of specific embodiments of our invention, it will be understood that these embodiments are merely for the purpose of illustration and description and that various other forms may be devised within the scope of our invention, as defined in the appended claims.

We claim:

1. Age-hardenable austenitic steel containing sufficient metal from the group consisting of manganese, up to 12% nickel and a mixture thereof, to render the steel substantially wholly austenitic characterized by the absence of tungsten and containing in addition thereto about .25 to 1% carbon, about .30 to 3% vanadium, and about 1 to 4% molybdenum.

2. Age-hardenable austenitic steel containing sufficient metal from the group consisting of manganese, up to 12% nickel and a mixture thereof, to render the steel substantially wholly austenitic characterized by the absence of tungsten and containing in addition thereto about .25 to 1% carbon, about .75 to 3% vanadium, 0 to 20% chromium and about 1 to 4% molybdenum.

3. Age-hardenable austenitic steel containing sufficient metal from the group consisting of manganese, up to 12% nickel and a mixture thereof to render the steel substantially wholly austenitic and containing in addition thereto about .25 to 1% carbon, about .30 to 3% vanadium and about 1.2 to 4% aluminum.

4. Age-hardenable austenitic steel containing sufficient metal from the group consisting of manganese, up to 12% nickel and a mixture thereof, to render the steel substantially wholly austenitic and containing in addition thereto about .40 to 1% carbon, about .40 to 3% vanadium and 3 to 4% aluminum.

5. Heat-treatment hardened austenitic steel articles containing sufficient metal from the group consisting of manganese, up to 12% nickel and a mixture thereof to render the steel substantially wholly austenitic and in addition thereto between about .25 to 1% carbon, about .30 to 3.00% vanadium and about 1.2 to 4% aluminum, said steel being age-hardened by solution annealing at a sufficiently high temperature for a long enough time to place the vanadium carbides in solution and cooling followed by aging at a temperature between 1100 and 1500° F.

6. Heat-treatment hardened austenitic steel articles, having a minimum DPH hardness of 300 containing sufficient metal from the group consisting of manganese, up to 12% nickel and a mixture thereof to render the steel substantially wholly austenitic and in addition thereto between about .40 to 1% carbon, about .40 to 3.00% vanadium and about 3 to 4% aluminum, said steel being age-hardened by solution annealing at a sufficiently high temperature for sufficient time to place the vanadium carbides in solution and cooling followed by aging at a temperature between 1100 and 1500° F.

7. Heat-treatment hardened austenitic steel articles containing sufficient metal from the group consisting of manganese, up to 12% nickel and a mixture thereof to render the steel substantially wholly austenitic and in addition thereto between about .40 to 1% carbon, about .40 to 3.00% vanadium, 0 to 20% chromium, 0 to 4% molybdenum, about 1.2 to 4% aluminum with the balance iron and elements in amounts which do not adversely affect the properties, said steel being age-hardened by solution annealing for sufficient times at a sufficiently high temperature and cooling followed by aging at a temperature between 1100 and 1500° F.

8. Age-hardenable austenitic steel containing sufficient metal from the group consisting of manganese, up to 12% nickel and a mixture thereof to render the steel substantially wholly austenitic and containing in addition thereto

about .25 to 1% carbon, about .30 to 3% vanadium, 0 to 20% chromium, 0 to 4% molybdenum and 1.2 to 4% aluminum.

9. Heat-treatment hardened austenitic steel articles containing sufficient metal from the group consisting of manganese, up to 12% nickel and a mixture thereof to render the steel substantially wholly austenitic and in addition thereto between about .25 to 1% carbon, about .30 to 3.00% vanadium, 0 to 20% chromium, 0 to 4% molybdenum and 1.2 to 4% aluminum, said steel being hardened by solution annealing at a sufficiently high temperature for sufficient time to place the vanadium carbides in solution and cooling followed by aging at a temperature between 1100 and 1500° F.

References Cited in the file of this patent

UNITED STATES PATENTS

|           |              |                |
|-----------|--------------|----------------|
| 1,106,207 | Guillaume    | Aug. 4, 1914   |
| 2,153,906 | Aborn et al. | Apr. 11, 1939  |
| 2,523,917 | Payson       | Sept. 26, 1950 |

FOREIGN PATENTS

|         |               |               |
|---------|---------------|---------------|
| 409,411 | Great Britain | May 3, 1934   |
| 507,591 | Belgium       | Dec. 31, 1951 |
| 518,985 | Belgium       | Apr. 30, 1953 |
| 663,461 | Germany       | July 2, 1935  |
| 171,966 | Switzerland   | Dec. 1, 1934  |